

# UNITED STATES PATENT OFFICE.

MERL R. WOLFARD, OF CAMBRIDGE, MASSACHUSETTS, ASSIGNOR OF ONE-FOURTH TO LEROY A. AMES, OF SPENCER, MASSACHUSETTS, AND ONE-FOURTH TO EVERETT E. KENT, OF NEWTON, MASSACHUSETTS.

## COMPOSITION FOR RESISTING HEAT.

1,263,831.

Specification of Letters Patent. Patented Apr. 23, 1918.

No Drawing.

Application filed August 8, 1916. Serial No. 113,696.

To all whom it may concern:

Be it known that I, MERL R. WOLFARD, a citizen of the United States, residing at Cambridge, in the county of Middlesex and 5 State of Massachusetts, have invented new and useful Improvements in Compositions for Resisting Heat, of which the following is a specification.

This invention relates to improvements in 10 compositions of matter for resisting heat, without cracking or crumbling under severe conditions, and in methods of making the same. It has been developed more especially to meet the peculiarly strenuous conditions 15 which exist within the combustion chamber of a particular type of an internal combustion engine, burning liquid fuel, but it is applicable to many other uses, some of which are hereinafter suggested. It is especially 20 the object to provide a composition that can resist conditions where the temperature stresses are severe, and tend to break down the structure of the material exposed to them, either because of extreme temperature 25 differences between adjacent portions of the material, or because of such temperature differences acting on a material which must also withstand pressure. Periodic variations in the temperature of a material are known 30 to be especially difficult to withstand under extreme conditions. The life of material under such conditions appears to be more or less independent of the period of time between variations, but almost directly propor- 35 tional to the number of variations or periods. This fact has been partially recognized at least, for many years; that is, efforts have been made to keep the temperature in large engines approximately the same when not 40 operating as when operating; also the life of many furnace linings is estimated by the number of "heats" rather than by the duration of any particular "heat."

Also in many industrial fields a material 45 is required both to withstand pressure and at the same time to permit the flow of a considerable amount of heat through it. Thus, for example a confining wall may be exposed on one side to a furnace flame and be in contact on the other with water, as is the case in certain portions of a steam boiler or of 50 an internal combustion engine. Wherever, under these conditions, the pressure to be sustained is high, or the capacity of a retain-

ing vessel is large, and particularly if both 55 of these conditions coexist, the thickness of the wall of the vessel must be relatively great. This causes the temperature difference between one side of the wall and the other to be excessive and the resulting 60 stresses in the wall to become extreme. Sometimes it may be desirable to laminate the structure of such a wall, as where it is exposed to the flame, in such manner that the 65 lamina or layer is exposed independently of the pressure sustaining wall, and also may shield it from the extreme temperature of combustion. This laminated structure may be very useful wherever the space available 70 for combustion is positively restricted, or wherever it may be desirable to restrict it, in 75 which case the lamina in contact with the flame may be maintained at a glowing temperature. By this means the combustion of the more difficult fuels may be materially 80 improved. Reference is hereby made to my co-pending application for patent Serial Number 8829 in which one form of the invention herein set forth is shown and claimed in combination with certain elements of an internal combustion engine.

I have discovered that a certain amount of nickel alloyed with iron will make a product having characteristics which are adapted to withstand these conditions, and which, 85 so far as I am aware, are not possessed by the previously known material that is available for use under commercial conditions.

In the best form in which I have made 90 experiments I have found that a composition of about  $\frac{2}{3}$  nickel and  $\frac{1}{3}$  iron has qualities which fit it for attaining the above described results. My experiments however, show 95 that these proportions can be varied, so that I believe a proportion at least as low as  $\frac{1}{3}$  of nickel, or as high as  $\frac{2}{3}$  of nickel, the remainder being iron would be satisfactory. My experiments also indicate that while purity of the iron is not essential better results 100 are attained with small percentage of carbon. The alloy may be made by melting together the desired amount of nickel and of iron, according to methods usually employed in the art, and can be handled upon cooling from the molten state by the usual 105 methods of handling metals. It is a particular advantage of this alloy that it is to be cast in its desired form, and that when

so cast makes a product which is free in a marked degree from blow holes and other defects. Such castings have a firm, compact and homogeneous structure which may be 5 easily machined to any desired shape. In common with other metals it has the property of being tenacious at ordinary temperatures, but unlike other metals it retains a high degree of tenacity at high temperatures, and under conditions under which all 10 other commercially available metals known to me have failed. With respect to tenacity it is of course entirely different from materials such as porcelain and other earthen 15 substances, commonly called refractory, both because such substances are apt to be porous and so not adapted either to conduct or to confine gases under pressure, are always more or less fragile, are not easily shaped to 20 conform precisely to a machined surface, and also because they will crack and crumble under the influence of heat. The distinction is yet more marked when the composition of the invention is compared with any such 25 material under conditions in which the adjacent parts of an integral piece are subjected to widely different temperatures or to repeated heatings and coolings. The composition of the invention is in fact par- 30 ticularly useful where a material is desired, capable of withstanding fluid pressure and capable of withstanding widely different temperatures in closely adjacent regions, or of withstanding repeated heatings and cool- 35 ings. The well known advantage of metals as compared with earthy substances is largely due to the greater freedom from cracking and crumbling, but the composition of the invention has properties not pos- 40 sessed by any metal previously known to me. When this composition, and nickel, for ex- 45 ample, are tested under identical conditions, the nickel will crystallize and crack; or iron, for example, will oxidize; or monel metal, which is reputed for its heat re- 50 sisting qualities, will crack and break down very quickly, while the composition of the invention undergoes the test without dis- 55 cernible change, and the test may be repeated many times or for a long duration without its undergoing any discernible change, in strength or structure. Without knowing with certainty the chemical explanation for the novel results attained, I believe that it 55 may be that the nickel prevents oxidation of the iron, and the iron prevents crystalliza-

tion of the nickel. Whatever the explana- 60 tion may be, it appears that a rather wide variation may be made in the composition of the alloy while still producing a metal hav- 60 ing superior heat resisting qualities.

The composition of the invention can be applied to many uses in the arts. Some of these are hereinbefore suggested; but its uses are not limited to those particularly 65 mentioned, and it has qualities of value in various respects.

I claim as my invention:

1. A wall shaped and adapted to confine material at high temperature, comprising an 70 alloy of nickel and iron having an internal organization such as results from solidification from a liquid state in approximately its said shape, the nickel constituting about one third to two thirds of the whole. 75

2. A wall shaped and adapted to confine material, said wall being in a state of internal stress resulting from great temperature differences between adjacent parts thereof and being an alloy of nickel and iron sub- 80 stantially as described, the nickel constituting about one third to two thirds of the whole. 80

3. A device for confining material at high temperature comprising a metal container of 85 about one-third to two-thirds of nickel alloyed with iron, having a relatively low content of carbon and formed without rolling or hammering.

4. A device for confining material at high 90 temperature comprising a body having high heat resisting properties and being the result of the solidification of a molten union of iron and nickel of which about one third to two thirds is nickel in substantially the 95 form of the body without hammering or rolling, substantially as described.

5. A process of making a body for confining materials subject to an oxidizing flame of high temperature comprising the melt- 100 ing together of nickel and iron, the nickel constituting about one-third to two-thirds of the whole, pouring the molten mixture into a mold of approximately the shape of said body and allowing it to solidify therein. 105

Signed by me at Boston, Mass., this 4th day of August, 1916.

MERL R. WOLFARD.

Witnesses:

JOSEPH T. BRENNAN,  
EVERETT E. KENT.